

# UNITED STATES PATENT OFFICE.

WINTWORTH V. LANDER, OF NEWTON, MASSACHUSETTS, ASSIGNOR TO GENERAL INDURATING CORPORATION, A CORPORATION OF NEW YORK.

## METHOD OF FILLING AND INDURATING POROUS MATERIAL AND THE PRODUCT THEREOF.

1,278,943.

No Drawing.

Specification of Letters Patent. Patented Sept. 17, 1918.

Application filed November 8, 1915. Serial No. 60,369.

To all whom it may concern:

Be it known that I, WINTWORTH V. LANDER, citizen of the United States, and resident of Newton, in the county of Middlesex 5 and State of Massachusetts, have invented new and useful Improvements in Methods of Filling and Indurating Porous Material and the Product Thereof, of which the following is a specification.

10 This invention relates to a method of filling and indurating porous material such as fiber board, or other fibrous or granular material, and also to a method of both indurating and waterproofing such material, and to 15 the resulting product.

The type of porous material which I prefer to use, is that made of fibers, and may be made by any suitable method. Particularly, I recommend wood pulp for making 20 the board, sheet, article or body to be treated, of whatever shape may be desired. Such material is porous and absorbent, and although possessing little inherent strength or hardness, is cheap and admirably adapted to my process. The fibrous material may be composed of a uniform and homogeneous mass of fibers throughout, or it may be built up of layers of fiber boards held together by a suitable cement or binder, such 25 as silicate of soda.

30 The method consists in filling the porosities or interstices of the material, whether it be fibrous or granular, with an elastic cementitious filler comprising a gum or resin, such as common rosin, and the residue from 35 the distillation of petroleum, which is a yellowish brown jelly-like substance, the two being in such proportion that the resin preponderates over the petroleum residue, so that the resulting composition manifests the 40 hardness of the resin, qualified by the softer and lubricant petroleum residue to such extent that the composition does not manifest the brittleness which is characteristic of 45 resins. The composition is introduced into the porous or interstitial material by means of a solvent and carrier, such as gasolene. The composition and method herein described and claimed constitute a special instance of a composition and method more 50 comprehensively described and claimed in the application for patent filed by me on December 20, 1916, Serial No. 137,959. It is desirable that the mixture be used hot to

insure a sufficiently thin consistency for 55 effective penetration of the material. After thus filling the porosities, either through and through, or to the desired depth, the treated material is dried.

To describe with more particularity and detail the preferred exemplification of my method: I mix common rosin of any desired grade and gasolene, in the proportions of about 4 pounds of rosin to 1 gallon of gasolene (approximately 6 pounds). The gasolene 60 dissolves the rosin, any sediment or dirt settling to the bottom, and the clear solution, which is made cold or at normal temperature, is poured off. With this solution 65 is mixed crude petroleum residue (which is a jelly-like mass constituting a residue resulting from the various processes of refining petroleum oil) in the proportion of about 3 pounds of petroleum residue to the (approximately) 10 pounds of the solution, 70 and the mixture is then preferably heated.

The porous material to be treated is then 75 immersed in, or sprinkled with, the said mixture. The material to be treated is itself preferably heated before treatment and 80 treated while hot, so as not to cool the mixture before the penetration is effected. The hot mixture penetrates the porous and absorbent material, reaching and filling the interstices and porosities. It is important, 85

although it may not always be essential, that the mixture be used hot, otherwise it may be too thick and viscous readily to penetrate the pores. A good mode of performing the 90 process is to place the mixture in a deep vessel over a gas flame. After the material has gone completely into solution, the temperature is raised to the point of ebullition of the solvent and carrier. This tends to cause a distillation of the gasolene but the depth 95 of the vessel may be such that the gasolene vapors do not rise above the top of the vessel and escape in appreciable quantity, since the upper part of the vessel and the surface or layer of cool air above act as a condenser 100 to return the gasolene vapors to the solution.

The material to be treated when placed in the hot solution causes a more violent ebullition, which is probably due in large part to displacement of air from the porosities of the material, for the ebullition soon substantially subsides.

The treated material, when taken from the

solution and immediately removed from the vessel, retains a coating of the admixture of rosin and petroleum residue on its surfaces after evaporation of the gasolene. If, 5 however, the treated material is lifted out of the solution and suspended within the vessel and within the gasolene vapors, it is bathed by the condensed vapors. A very short bath of this sort removes the rosin and 10 petroleum residue from the surfaces, and the impregnated material then dries clean and free of surface coating when removed from the vessel.

The mixture of rosin, which is a brittle 15 gum, and petroleum residue, which is a viscous, heavy oil, produces a more or less elastic, pitch-like, cementitious substance, the friability of the rosin being tempered by the oil, and the viscosity of the oil being 20 tempered by the rosin; these substances are readily soluble in gasolene, and the solution penetrates the interstices of porous material. Subsequent evaporation of the gasolene leaves the more or less elastic pitch-like and 25 cementitious substance uniformly filling the porosities of the treated material.

If the material consists of a single, substantially homogeneous layer or mass, the mixture will penetrate and fill the porosities 30 very rapidly, an immersion of a few minutes being sufficient for boards or other articles not exceeding an inch in thickness. It will also be evident that if a penetration through and through is not desired, but only a surface treatment, the time of immersion may 35 be reduced. An instantaneous immersion will serve to indurate and waterproof the surface, forming what may be termed a rind.

If the porous material is of laminated 40 structure, the binding material which holds the layers together may tend to resist the penetration of the mixture and a longer immersion may be necessary, according to the thickness of the material, the number of 45 layers, and the resistance of the binder between the layers. But even if considerable resistance is offered between the layers the mixture will eventually penetrate through and through the article from the edges of 50 the layers.

After treatment as above described, the board or other article is freed from the carrier by evaporation either in the atmosphere at normal temperatures or by artificial heat.

55 The method may be varied by first mixing the rosin and petroleum residue, heating the same until it becomes a viscous mass, and then thinning with the gasolene. As, however, the rosin is more readily soluble 60 in gasolene than in the residue I prefer the procedure first set forth.

The rosin, or other gum or resin-like substance, mixed with the petroleum residue, forms a cement which is exceedingly hard 65 and tough, yet sufficiently plastic or elastic

so that it will not break under shocks and strains in use. Without such residue the rosin is too brittle to secure satisfactory induration of the porous material. The rosin mixed with the residue, carried by the solvent, also penetrates the porosities better than rosin alone in a solvent, or than rosin mixed with an oil which tends to oxidize, especially when heated, thereby forming a varnish which stops or retards penetration. 75

Gasolene is the best and most readily available solvent and carrier for the stated purpose with which I am acquainted. Its chief function is to thin the cementitious substance or mixture and carry it into the 80 pores, a function aided by heat, after which the gasolene evaporates, but instead of leaving porosities when the gasolene leaves the material, the spaces vacated by the gasolene are filled by the elasticity of the cementitious 85 filler, and by the tendency of the fibers of the material to draw together, the latter phenomenon being evidenced by the fact that the product in its finished condition is somewhat thinner, although filled with the 90 compound of rosin and the oil residue, than the untreated porous body was at the start.

All residues from the distillation of oils, do not have the same waterproofing effect, 95 although they have the same or a similar effect in preventing the rosin from becoming brittle and in aiding the cementitious compound to penetrate the pores. Petroleum residue, however, when mixed with the gum or resin-like substance, not only aids in the 100 induration of the porous body being treated but renders the product completely imperious to water or moisture.

The material thus treated is solid, homogeneous and dense throughout, the fibers are 105 hardened and compacted, and the product is tough, hard and strong. It is capable of holding screws and may be otherwise worked like wood. The oil affords a handsome finish, which may be readily polished, without the use of varnish or other finishing material, but the product is nevertheless perfectly adapted to painting, papering, or to other similar treatment if desired. The product has practically no tendency to expand or contract with variations in temperature or humidity; it is an admirable heat insulation; is not affected by moisture; possesses great breaking strength, tensile strength and tearing strength; and is substantially inflexible. It is capable of use for a great variety of purposes in place of wood and other materials, and is especially valuable in situations where resistance to heat and cold, indifference to moisture, strength 115 and durability are required.

Red or white rosin may be used, as desired, with a consequent difference in color of the finished product. Or artificial colorings may be used in the mixture, to obtain 120 125 130

a great variety of color effects in the finished article.

The petroleum residue which I preferably employ is an amorphous product generally known as crude petrodatum. It is obtained from paraffin-base petroleum such as obtained in Pennsylvania when refined by the process known as fractional distillation. It has a flash point of approximately 500° F, 10 a melting point of the order of 120° to 130° F, and is a mixture of saturated and unsaturated hydrocarbons. The residue comprises olefins, naphthenes, and paraffins in amorphous form, but contains no paraffin as such, 15 that is, no paraffin in crystalline commercial form. Most of the paraffin is removed from the crude petroleum in the form of paraffin wax before the residue which I employ is arrived at.

20 I claim:

1. The method of treating porous material, whether fibrous or granular, which consists in filling the porosities of the material with a filler comprising a resin and petroleum residue dissolved in an evaporable carrier, the amount of resin being at least of the order of the amount of petroleum residue, and thereafter removing the carrier from the material by evaporation.

2. The method of indurating porous material, whether fibrous or granular, which consists in impregnating it with an evaporable solution of a cementitious filler comprising a resin and petroleum residue, the 30 amount of resin being at least of the order of the amount of petroleum residue, at a temperature approximating to the boiling point of the evaporable solvent, and thereafter removing the solvent from the material by evaporation.

3. The method of indurating porous material, whether fibrous or granular, which consists in impregnating it with a solution of a cementitious filler comprising a resin and petroleum residue in an evaporable solvent, bathing the surface of the impregnated material in vapor of the solvent, and thereafter removing the solvent from the material by evaporation.

4. The method of indurating porous material, whether fibrous or granular, which consists in filling the porosities of the material with a cementitious filler comprising a gum or resin-like substance and a residue 55 from the distillation of oils, dissolved in a suitable solvent and carrier, thereafter bathing the surface in the condensing vapors of the carrier, and thereafter removing the carrier from the porosities by evaporation.

5. Porous material, whether fibrous or granular, having its porosities impregnated

with a composition of a resin and petroleum residue wherein the former predominates.

6. The method of indurating porous material, whether fibrous or granular, which consists in filling the porosities of the material with a cementitious filler comprising a resin and petroleum residue wherein the former predominates, dissolved in gasoline, and thereafter removing the gasoline from the material by evaporation.

7. The method of indurating porous material, whether fibrous or granular, which consists in impregnating it with an evaporable solution in gasoline, of a cementitious 75 filler comprising a resin and petroleum residue wherein the former predominates, at a temperature approximating to the boiling point of the evaporable solvent, and thereafter removing the gasoline from the material by evaporation.

8. The method of indurating porous material, whether fibrous or granular, which consists in impregnating it with a solution of a cementitious filler comprising a resin 85 and petroleum residue in gasoline, bathing the surface of the impregnated material in vapor of the gasoline, and thereafter removing the gasoline from the material by evaporation.

9. An article of manufacture comprising fiber board indurated with a composition of resin and petroleum residue in which the amount of resin is at least of the order of the amount of petroleum residue.

10. The method of treating porous material which comprises impregnating the material with a solution comprising resin and petroleum residue in an evaporable carrier, and thereafter bathing the surface of the impregnated material in vapor of the solution.

11. The method of treating porous material which comprises impregnating the material with a composition comprising resin and petroleum residue in an evaporable carrier, bathing the surface of the impregnated material in vapor of the carrier, and thereafter removing the carrier from the material.

12. The method of treating porous material which comprises impregnating the material in a filling solution comprising a volatile solvent and at a temperature sufficient to give off a vapor, and thereafter bathing the surface of the impregnated material in the vapor of the solution under such conditions as to remove the filling matter from the surface of the material.

Signed by me at Boston, Massachusetts, this 5th day of November, 1915.

WINTWORTH V. LANDER.